

H. P. BROWN.

COMPOSITION OF MATTER TO RESIST WEAR AND ANTI SKID DEVICE EMBODYING THE SAME.  
APPLICATION FILED FEB. 7, 1914.

1,266,100.

Patented May 14, 1918.

Fig. 1.



Fig. 2.



Fig. 3.



Fig. 4.



Fig. 5.



Fig. 6.



Fig. 7.



Fig. 8.



Fig. 10.



Witnesses:

*H. P. Brown*

Ella Hammerchlag

Harold P. Brown

Inventor

By his Attorney

*Robert G. Brannigan*

# UNITED STATES PATENT OFFICE.

HAROLD P. BROWN, OF NEW YORK, N. Y.

## COMPOSITION OF MATTER TO RESIST WEAR AND ANTISKID DEVICE EMBODYING THE SAME.

1,266,100.

Specification of Letters Patent.

Patented May 14, 1918.

Application filed February 7, 1914. Serial No. 817,271.

To all whom it may concern:

- Be it known that I, HAROLD P. BROWN, a citizen of the United States, residing in the city of New York, county and State of New York, have invented certain new and useful Improvements in Composition of Matter to Resist Wear and Antiskid Devices Embodying the Same, of which the following is a full, clear, and accurate specification.
- 10 This invention relates to composition of matter especially designed to resist wear, to act as an abradant or to offer high resistance to slippage. By high resistance to slippage is meant a high coefficient of friction. This invention also relates to the embodying of such composition of matter in vehicle tires, abrasive devices, step treads, shoe heels and the like.
- 15 This invention has in view the embedding of abrasive, friction or wear material in a sub-divided state in an elastic matrix such as rubber.
- 20 At the present time it is known to be old to use abrasive material of the nature of emery, carborundum and the like embedded in soft metal of low melting point in places where an abrasive or friction material is needed. It is also old to plate the surface of such abrasive material with metal so that
- 25 the matrix metal will adhere to such plating. The lack of elasticity in such metal matrix, however, causes the enlargement of the setting and the displacement and loss of the abrasive material.
- 30 An abrasive material has also been used with rubber in shoe soles and with rubber for erasers, but no method has heretofore been discovered for causing a strong adhesion between the surfaces of the abrasive and the rubber. The abrasive has merely been mechanically mixed with the rubber and under the strain of compression and extension in service it works out and is lost.
- 35 In rubber automobile tires, spool shaped buttons or rivets have been inserted radially in the rubber to obtain friction on a greasy road. These spools or rivets have sometimes been cemented into place, but in warm weather the heating of the metal causes its surface to slip on the contiguous rubber sur-

face so that the metal is forced out from the tire and lost.

This difficulty is overcome in this invention by plating or coating the surfaces of the particles of the abradant, friction or wear material with an alloy which has the property of adhering tightly to rubber or similar elastic materials when the latter is vulcanized preferably under more or less pressure. Such an alloy may be made of copper, zinc and antimony used in an electro-plating bath with a solution which will dissolve it.

Steel containing 11% to 13% of manganese is so strongly wear resisting that it cannot be shaped by machine tools or files. It is therefore an excellent material for withstanding heavy blows and great weight without injury. On the other hand, emery, 65 silex, corundum, or carborundum while fine abradants and excellent in preventing slippage, may be crushed by too heavy weights or blows. Therefore in my invention, it is intended to use particles of special 70 manganese steel to take the heavy weights and particles of abradant material preferably of the same size or smaller embedded in the same soft rubber to supply the anti-skidding and non-slipping feature where 75 the service is such as to require it.

Part of my invention consists in embodying in a special way this material in articles such as stair treads, vehicle tires or anti-skid devices, grinding wheels, tools and the like.

The material *per se* needs no illustration.

In the accompanying drawing forming

part of this specification:

Figure 1 is a cross section of the tread 90 such as a step tread.

Fig. 2 is a cross section of such pneumatic vehicle tire. The invention applies equally well to other types of tires.

Fig. 3 is a cross section on line III—III 95 of Fig. 4 showing a tire equipped with an anti-skid device embodying this invention.

Fig. 4 is a plan view of the same.

Fig. 5 is medial cross section through such a grinding or polishing wheel.

Fig. 6 is a vertical section through such a shoe sole.

Fig. 7 is a vertical section through such a shoe heel.

Fig. 8 is a longitudinal cross section of the ordinary anti-skid tire chain equipped with the gripping and wear resisting material.

Fig. 9 is a view of a modified structure, and

Fig. 10 is a view of a second modified structure.

Referring to Fig. 1, the base B of the tread consists of a metal or other firm plate, which is plated with the above mentioned alloy or one similar to it indicated at P; next is placed a layer of elastic rubber or similar material R; having an exterior layer D in which are inserted particles of the slip preventing material A, A each particle of which is completely covered with a layer of the said plating. After this compound tread is vulcanized, the rubber adheres strongly but flexibly to the base B and to each particle. The layer R acts as a cushion preventing the wear resisting particles from acting injuriously upon the base B; it also when under pressure tends to push outward the particles A into the contacting surface, thereby preventing slippage.

X represents any known type of reinforcement. Such reinforcement is applied either to the wear resisting material D or to the cushion member R or both as occasion demands. If necessary, such reinforcement may be added to other structures disclosed herein. If required plated wear resisting particles W, W may also be inserted in the material D.

Referring to Fig. 2, R' is a conventional pneumatic tire, the outer layer D' of which contains the plated wear resisting particles W. Gripping particles A may be added. C is the reinforcing metal cable or wire plated with the said alloy to secure greater adhesion to the tire. In the case of solid tires similar reinforcing treads and cables may be used.

Referring to Figs. 3 and 4, R<sup>2</sup> is a conventional tire and S the anti-skid device applied to the tread thereof. The anti-skid device is composed of a metal base plate B' provided with hook or loop H, H at each end, and plated with the alloy and coated on the face in contact with the tire with rubber or similar material R<sup>3</sup>. R<sup>4</sup> is a coating of rubber or similar material on the exterior of the face. D<sup>2</sup> is a tread containing the wear resisting particles W, W and the slip preventing particles A, A all inclosed in the said plating P and therefore after vulcanization, adhering strongly but flexibly to the elastic rubber. The anti-skid device so composed may be made as illustrated in Figs. 3 and 4 of a series of

diamond shaped plates bent around the exterior of the tire and held in place by suitable securing means to a ring or endless spring G on each side of the tire. These plates may be arranged in contact as illustrated in Fig. 4 or they may be overlapped as shown in Fig. 9, thus giving increased friction or driving surface. The anti-skid device may be also composed of bands placed across the tire a few inches apart as shown in Fig. 10, such bands being secured to wire rings on either side of the tire by bending over the ends.

Referring to Fig. 5, E is a grinding or polishing disk having an alloy plating P and the two layers R<sup>5</sup> and R<sup>6</sup> of rubber, containing particles A, A of the abradant material. Of course the entire grinding or polishing device may be of the abradant material, as best suits the need of the user.

Referring to Fig. 6, F is a portion of 85 shoe showing the sole in a transverse vertical section. In this I is the usual inner sole. R' the inner layer of flexible material. D<sup>8</sup> the outer layer of elastic material having embedded therein plated wear 90 resisting or gripping particles W and A.

Referring to Fig. 7, J is the rear elevation of the shoe with the heel portion in vertical section. I' is the inner sole or one of the intermediate heel lifts. R<sup>9</sup> the flexible cushion layer and D<sup>9</sup> the elastic outer layer having the plated wear resisting and gripping particles W and A embedded therein.

Referring to Fig. 8, K represents the tire 100 in longitudinal section; L the ordinary anti-skid tire chain member passing laterally across the tread of the tire. M, is a link of the chain plated with the alloy. R<sup>10</sup> the mass of rubber or similar elastic material embracing the link; D<sup>10</sup> a layer of rubber or similar elastic material having embedded therein the wear resisting and gripping particles W and A coated with the alloy. It will be seen that the tire 110 chain so equipped presents a soft, non-chafing surface to the tire and a gripping and wear resisting surface to the roadway.

It is to be appreciated that any attempt to embed sub-divided wear-resisting, abrasive or gripping material directly or by means of any hitherto known cements, results in failure because of insufficient bond. This is aggravated in cases where the material is subjected to heat, since heat softens 115 the cement. By connecting the elastic matrix and the wear-resisting, abrasive or gripping material with the alloy plating, a stronger bond results, which is often superior to the cohesion of the bodies joined. 120 The resulting flexible, wear-resisting abrasive or gripping material has certain valuable properties. In the case of rigid mate-

rials of this nature when subjected to duty the wear-resisting, abrasive or gripping particles in contact with the object acted upon are subjected to excessive pressure, 5 and as they are often of a crystalline nature, they crumble so that the material wears rapidly. With this elastic material it can be seen that the abrasive wear-resisting or gripping material is held up to its work but 10 that the pressure is not unyielding so that while the particles perform their designed duty they are given an opportunity to yield to excessive force.

It is also appreciated that while in any of 15 these structures the cushion R is of advantage, its use is not essential in all cases in my invention. Where desirable, the material bearing the abradant, gripping or wear resisting material may be attached directly 20 to the base.

In the claims, the term hard material is understood as representing materials having abrasive, wear-resisting and gripping properties.

25 By the expression of material in a state of sub-division I do not intend to be limited to any particular size.

I claim:

1. The combination of a hard material in 30 a state of sub-division firmly adhering to an elastic matrix by result of chemical combination between the material and the matrix.

2. The combination of a wear-resisting 35 material in a state of sub-division firmly adhering to an elastic matrix by result of chemical combination between the material and the matrix.

3. The combination of an abrasive or 40 gripping material in a state of sub-division firmly adhering to an elastic matrix by result of chemical combination between the material and the matrix.

4. The combination of a hard material in 45 a state of sub-division firmly united to an elastic matrix and the matrix firmly united to a base by result of chemical combination between the said material, the base and the matrix.

50 5. The combination of a wear-resisting material in a state of sub-division firmly adhering to an elastic matrix and the matrix firmly united to a base by result of chemical combination between the said material, the base and the matrix.

55 6. The combination of an abradant or gripping material in a state of sub-division firmly united to an elastic matrix and the matrix firmly adhering to the base by result of chemical combination between the said material, the base and the matrix.

60 7. The combination of a hard material in a state of sub-division firmly adhering to an elastic matrix by an interposed plating.

8. The combination of a hard material in a 65 state of sub-division, a plating applied to such material, an elastic matrix embracing such plated material, a base member and a cushion interposed between the base and the matrix.

70 9. The combination of a wear resisting material in a state of sub-division, a plating applied thereto, an elastic matrix embracing such plated material, a base member and a cushion interposed between the base 75 and the matrix.

10. The combination of an abradant or gripping material in a state of sub-division, a plating applied to such material, an elastic matrix embracing such plated material, 80 a base member and a cushion interposed between the base and the matrix.

11. The combination of a hard material in a state of sub-division; plating applied to such material; an elastic matrix embracing such plated material and an elastic cushion applied to a portion of said matrix.

12. The combination of a wear resisting material in a state of sub-division; plating applied to such material; an elastic matrix 90 embracing such plated material and an elastic cushion applied to a portion of said matrix.

13. The combination of an abradant or gripping material in a state of sub-division; 95 plating applied to such material; an elastic matrix embracing such plated material and an elastic cushion applied to a portion of said matrix.

14. The combination of a hard material 100 in a state of sub-division; plating applied to such material; an elastic matrix embracing such plated material and a reinforcement embedded in such elastic matrix.

15. The combination of a wear resisting 105 material in a state of sub-division; plating applied to such material; an elastic matrix embracing such plated material; and a reinforcement embedded in such elastic matrix.

16. The combination of an abradant or 110 gripping material in a state of sub-division; plating applied to such material; an elastic matrix embracing such plated material; and a reinforcement embedded in such elastic matrix.

115 17. The combination of a hard material in a state of sub-division, plating applied to such material; an elastic matrix embracing such plated material; a reinforcement embedded in such elastic matrix and a base member secured to said matrix.

18. The combination of a wear resisting material in a state of sub-division; plating applied to such material; an elastic matrix embracing such plated material; a reinforcement embedded in such elastic matrix and a base member secured to said matrix.

125 19. The combination of an abradant or

gripping material in a state of sub-division; plating applied to such material; an elastic matrix embracing such plated material; a reinforcement embedded in such elastic matrix and a base member secured to said matrix.

20. The combination of a hard material in a state of sub-division; plating applied to such material; an elastic matrix embracing such plated material and an elastic cushion applied to a portion of said matrix, and a reinforcement embedded in the resulting elastic structure.

21. An elastic tire comprising a tread element composed of elastic matrix and plated hard material in a state of sub-division embedded in said matrix.

22. An anti-skid device for tires or the like, comprising a base member, an elastic cushion applied to both sides of the base, an

elastic matrix applied to the exterior of the cushion and hard plated material in a state of sub-division embedded in said matrix.

23. An element of anti-skid device, comprising a chain, an elastic cushion embracing such chain, an elastic matrix applied to portion of said cushion, a hard plated material in a state of sub-division embedded in such elastic matrix.

24. The combination of a hard material in a state of sub-division, a surrounding elastic matrix a uniting material interposed between the hard material and matrix which has greater adhering properties to both the hard material and the matrix than does the hard material to the matrix.

HAROLD P. BROWN.

Witnesses:

JOHN COMERY,  
E. M. REED.

Copies of this patent may be obtained for five cents each, by addressing the "Commissioner of Patents, Washington, D. C."